# EUROPEAN PATENT SPECIFICATION

(11) **EP 3 081 662 B1**
(45) Date of publication and mention of the grant of the patent: **13.11.2019**
(21) Application number: 14869973.9
(22) Date of filing: 10.12.2014
(51) Int. Cl.: C21D 8/02, C21D 9/46, C21D 9/50, C22C 38/00, C22C 38/02, C22C 38/04, C22C 38/06, C22C 38/08, C22C 38/12, C22C 38/14, C22C 38/16, C22C 38/42, C22C 38/44, C22C 38/46, C22C 38/48, C22C 38/50, C22C 38/54, C22C 38/58

(54) **STEEL PLATE AND METHOD FOR MANUFACTURING SAME**
STAHLPLATTE UND VERFAHREN ZUR HERSTELLUNG DAVON
TÔLE D'ACIER ET PROCÉDÉ PERMETTANT DE FABRIQUER CETTE DERNIÈRE

(30) Priority: 12.12.2013 JP 2013257401
(43) Date of publication of application: 19.10.2016
(73) Proprietor: JFE Steel Corporation, Tokyo 100-0011 (JP)
(72) Inventor: ICHIMIYA, Katsuyuki, Tokyo 100-0011 (JP); KITSUYA, Shigeki, Tokyo 100-0011 (JP); HASE, Kazukuni, Tokyo 100-0011 (JP); ENDO, Shigeru, Tokyo 100-0011 (JP)
(74) Representative: Grünecker Patent- und Rechtsanwälte PartG mbB
(86) International application number: PCT/JP2014/083321
(87) International publication number: WO 2015/088040

(56) References cited:
- WO-A1-2008/078917
- WO-A1-2013/118313
- WO-A1-2013/145770
- CN-A- 102 691 015
- JP-A- 2001 247 932
- JP-A- 2005 281 842
- JP-A- 2006 291 349
- JP-A- 2009 263 777
- JP-A- 2009 263 777
- JP-A- 2013 151 732
- US-A1- 2010 074 794

## Description

### TECHNICAL FIELD

This disclosure relates to a high tensile strength steel plate, and a method for manufacturing the same, used in steel structures such as marine structures and ships, pressure vessels, and penstocks. In particular, this disclosure relates to a thick, high tensile strength steel plate, and a method for manufacturing the same, that not only has a yield stress (YS) of 460 MPa or greater and excellent strength and toughness, but that also has excellent low-temperature toughness in a multilayer weld (CTOD property) and that, after Post Weld Heat Treatment (PWHT), has excellent strength and toughness (PWHT property).

### BACKGROUND

Steel plates used in ships, marine structures, pressure vessels, and the like are subjected to welding to form structures with desired shapes. Therefore, from the perspective of structural safety, these steel plates are not only required to have high strength and excellent toughness but also to have excellent toughness in weld joints (weld metal and Heat-Affected Zone (HAZ)) upon welding.

The absorbed energy by a Charpy impact test has mainly been used as the basis for evaluating the toughness of steel plates. In recent years, however, a Crack Tip Opening Displacement test (CTOD test) has often been used for greater reliability. This test evaluates the resistance to occurrence of brittle fracture by forming a fatigue precrack in a test piece at the location to be evaluated for toughness, subjecting the test piece to three-point bending, and measuring the amount of the crack opening (plastic deformation volume) immediately before fracture.

Since a fatigue precrack is used in a CTOD test, an extremely small region is evaluated for toughness. Therefore, if a local brittle zone exists in the steel plate, a low toughness may in some cases be indicated by the CTOD test, even if a good toughness is obtained with a Charpy impact test.

In a thick steel plate or the like, local brittle zones easily occur in the heat-affected zone, which is subjected to a complicated thermal history due to multilayer welding. In addition, the bond (the boundary between weld metal and base material) and a region in which the bond is formed into a dual phase region by reheating (a region in which coarse grains are formed in the first cycle of welding and which is heated into a ferrite and austenite dual phase region by the subsequent welding pass, hereinafter referred to as a dual phase reheating area) are also prone to becoming local brittle zones.

Since the bond is exposed to a high temperature just below the melting point at the time of welding, austenite grains are coarsened and are likely to be transformed, by the subsequent cooling, into an upper bainite structure that has a low toughness. Therefore, the toughness of the matrix itself tends to reduce. Furthermore, brittle structures such as a Widmanstatten structure or isolated martensite (also referred to as M-A) easily occur. If such a brittle structure occurs, the toughness of the steel plate tends to reduce even further.

In order to improve the toughness of the heat-affected zone, for example a technique that incorporates TiN in the steel plate by fine particle distribution to reduce coarsening of austenite grains and to create ferrite nucleation sites has been put to practical use. The bond, however, may be heated to a temperature region at which TiN dissolves. As the demand for low-temperature toughness becomes more stringent, the heating temperature rises, thus making it more difficult to obtain the above-described effect from fine particle distribution of TiN.

To resolve these problems, JP H03-053367 B2 (PTL 1) and JP S60-184663 A (PTL 2) disclose techniques in which, by dispersing fine grains in steel plates by means of combined addition of rare-earth elements (REM) and Ti, grain growth of austenite is suppressed, thereby improving the toughness of the weld zone.

PTL 1 and PTL 2 also disclose a technique for dispersing Ti oxides, a technique for combining the capability of ferrite nucleation of BN with oxide dispersion, a technique for adding Ca and a REM to control the morphology of sulfides so as to increase the toughness, and other such techniques.

JP 3697202 B2 (PTL 3) discloses a technique for dispersing Ti oxides into steel so as to improve the HAZ toughness.

Furthermore, in the dual phase reheating area, carbon becomes concentrated in a region where reverse transformation to austenite occurs due to dual phase reheating, and brittle bainite structures including isolated martensite are generated during cooling, resulting in reduced toughness of the steel. To avoid this reduction in toughness, techniques have been disclosed to reduce the contents of C and Si in the chemical composition, inhibit the generation of isolated martensite, and improve the toughness, and to ensure the base material strength by adding Cu (for example, JP 3045856 B2 (PTL 4) and JP 4432905 B2 (PTL 5)).

The technique disclosed in PTL 4 sets the cooling rate after rolling to 0.1 °C/s or less and adopts a method to precipitate Cu particles during this process. Such a technique is problematic, however, in terms of manufacturing stability.

With the technique disclosed in PTL 5, the N/A1 ratio is set between 0.3 and 3.0, thereby suppressing toughness degradation due to the adverse effect of coarsened AlN and of solute N, but it is easier to control solute N with Ti.

In thick material for which YS exceeds 460 MPa, Post Weld Heat Treatment (PWHT) may be applied. During PWHT, the base material is also heated at the same time. Therefore, the base material properties need to be maintained even upon PWHT. Conventionally, in order to control a reduction in strength due to heat, an element that forms a precipitate at that temperature is generally added.
A further steel plate having a low yield ratio and high strength excellent in terms of strain ageing resistance and a method for manufacturing the same is disclosed in PTL 6.

### CITATION LIST

### Patent Literature

PTL 1: JP H03-053367 B2
PTL 2: JP S60-184663 A
PTL 3: JP 3697202 B2
PTL 4: JP 3045856 B2
PTL 5: JP 4432905 B2
PTL 6: WO2013/145770 A1

### SUMMARY

### (Technical Problem)

The techniques disclosed in PTL 1 and PTL 2 target relatively low strength steel material with a small amount of alloying elements. Unfortunately, these techniques cannot be applied to higher strength, thick material with a large amount of alloying elements, since the HAZ structure does not include ferrite.

With the technique disclosed in PTL 3, it is difficult to incorporate Ti oxides stably into steel by fine particle distribution.

Furthermore, ensuring strength by Cu precipitates often leads to a reduction in toughness, causing problems for ensuring the low-temperature toughness of the steel plate. In steel material that uses strengthening by Cu precipitation as recited in PTL 5, Cu particles also grow large during the PWHT, causing the problem of the strength tending to reduce.

Additionally, in recent years, steel structures such as ships, marine structures, pressure vessels, and penstocks have increased in size, leading to a desire for even higher strength steel.

The steel material used in these steel structures is often thick material, for example with a plate thickness of 35 mm or greater. Therefore, in order to ensure a strength such that the yield stress is at least 460 MPa grade, a steel chemical composition including a large amount of added alloying elements has become advantageous.

Sufficient examination has not been made, however, of how to improve toughness of the bonds and the dual phase reheating areas in high tensile strength steel material with a large amount of alloying elements. As for ensuring base metal properties after PWHT, it is difficult to maintain strength and toughness by simply adding precipitating elements as in conventional techniques.

Therefore, it would be helpful to provide thick, high tensile strength steel, and a method for manufacturing the same, that is suitable for use in steel structures such as marine structures, ships, pressure vessels, and penstocks, has a yield stress (YS) of 460 MPa or greater (satisfying this level of YS is referred to as high tensile strength in this disclosure), and has excellent low-temperature toughness of the heat-affected zone in a multilayer weld (CTOD property) and excellent strength and toughness after Post Weld Heat Treatment (PWHT property).

### (Solution to Problem)

To that end, we engaged in intensive studies and made the following discoveries.
(a) Since the CTOD property is evaluated with a test piece having the entire thickness of the steel plate, the central segregation area where components are concentrated becomes the origin of fracture.
   Consequently, in order to improve the CTOD property of the heat-affected zone, it is effective to control elements that easily concentrate as central segregation of the steel plate to a proper amount, thereby suppressing the hardening of the central segregation area. Furthermore, at the center of the slab, which is the last portion to solidify when the molten steel solidifies, the concentration of C, Mn, P, Ni, and Nb is higher than the concentration of other elements. Hence, it is effective to control the added amounts of these elements on the basis of the central segregation area hardness index, thereby reducing the hardness at the central segregation area.
(b) In order to improve the toughness of the heat-affected zone, it is effective to use TiN efficiently to suppress coarsening of the austenite grains in the vicinity of the weld bond. In particular, by controlling the Ti/N ratio to an appropriate level, TiN can be uniformly and finely dispersed in the steel.
(c) It is effective to use crystallization of the Ca compound (CaS), which is added for morphological control of sulfides, to improve the toughness of the heat-affected zone.
   Since CaS crystalizes at a low temperature as compared to oxides, CaS can be distributed uniformly as fine particles. Furthermore, by controlling the amount of Ca added and the amount of dissolved oxygen in the molten steel at the time of addition to be within appropriate ranges, solute S can also be guaranteed after CaS crystallization. Hence, MnS precipitates on the surface of the CaS to form a complex sulfide. Since a Mn dilute zone is formed around the MnS, ferrite transformation is further promoted.
(d) In addition to Nb, which forms precipitates, adding Ti and Mo as essential elements allows formation, at the stage of manufacturing a steel plate, of fine precipitates of a complex carbonitride of Mo, Ti, and Nb, which does not coarsen even when subjected to heating by PWHT (performed in a range of approximately 550 °C to 650 °C for 2 h to 4 h).

Conventionally, the reduction in strength after PWHT in a steel plate exceeding YS: 460 MPa grade is significant, but in a developmental steel plate, we discovered that by the stable existence of fine Mo, Ti, Nb complex precipitates (carbides, nitrides, or carbonitrides), strengthening by precipitation can be maintained, and the reduction in strength of the steel plate can be suppressed. Furthermore, due to the existence of fine Mo, Ti, Nb complex precipitates, the toughness of the steel plate can also be maintained.

This disclosure was completed based on the above discoveries, and the primary features thereof are as defined in the claims.

### (Advantageous Effect)

According to this disclosure, a thick, high tensile strength steel plate, and a method for manufacturing the same, that is suitable for use in large steel structures such as marine structures, has a yield stress (YS) of 460 MPa or greater, and has an excellent CTOD property in a multilayer weld and an excellent PWHT property can be obtained. Therefore, this disclosure is extremely useful in industrial terms.

### BRIEF DESCRIPTION OF THE DRAWINGS

In the accompanying drawings:
FIG. 1 illustrates the relationship between change in strength/toughness and the precipitate size/composition during PWHT; and
FIG. 2 illustrates TEM replica observation and EDX analysis results for precipitates in a steel plate.

### DETAILED DESCRIPTION

Our methods and products will be described in detail below.

First, reasons why the chemical composition (steel composition) of the steel plate (also referred to as thick material) has been restricted to the aforementioned ranges will be described in detail for each element. The % representations below indicating the chemical composition of the steel plate are in mass% unless stated otherwise.

### C: 0.020 % to 0.090 %

C is an essential element for ensuring the strength of a high tensile strength steel plate. When the C content is less than 0.020 %, quench hardenability is degraded, and it becomes necessary to add a large amount of quench hardenability-improving elements, such as Cu, Ni, Cr, or Mo, in order to ensure strength, resulting in a rise in costs. Conversely, when the amount of C added exceeds 0.090 %, the toughness of the weld zone degrades. Therefore, the C content is set in the range of 0.020 % to 0.090 %, and preferably 0.020 % to 0.080 %.

### Si: 0.01 % to 0.35 %

Si is added as a deoxidizing element and in order to obtain the steel plate strength. To obtain these effects, the Si content needs to be at least 0.01 %. On the other hand, a large Si content exceeding 0.35 % leads to deterioration in weldability and toughness of the weld joint. Therefore, the Si content needs to be set in the range of 0.01 % to 0.35 %, preferably 0.01 % to 0.23 %.

### Mn: 1.40 % to 2.00 %

In order to ensure the steel plate strength and the weld joint strength, the Mn content needs to be at least 1.40 %. Conversely, when the amount of Mn content exceeds 2.00 %, the weldability deteriorates, quench hardenability becomes excessive, and the toughness of the steel plate and the toughness of the weld joint deteriorate. Therefore, the Mn content is set in the range of 1.40 % to 2.00 %, more preferably 1.40 % to 1.95 %.

### P: 0.008 % or less

P, which is an impurity element, degrades the toughness of the steel plate and the toughness of the weld zone. In particular, when the P content in the weld zone exceeds 0.008 %, the CTOD property markedly degrades. Therefore, the P content is set to 0.008 % or less, preferably 0.006 % or less. The P content is preferably as small as possible, but considering factors such as refining cost, the lower limit may be approximately 0.002 %.

### S: 0.0035 % or less

S is an impurity element, and when the content thereof exceeds 0.0035 %, the toughness of the steel plate and the weld zone deteriorate. Therefore, the S content is set to 0.0035 % or less, preferably 0.0030 % or less. The S content is preferably as small as possible, but considering factors such as refining cost, the lower limit may be approximately 0.0004 %.

### Al: 0.010 % to 0.060 %

Al is an element to be added in order to deoxidize molten steel, and the Al content needs to be set to 0.010 % or more. When the Al content exceeds 0.060 %, however, the toughness of the steel plate and the toughness of the weld zone are degraded, and Al is mixed into the weld metal by dilution due to welding, which degrades toughness. Therefore, the Al content is limited to 0.060 % or less, preferably 0.017 % to 0.055 %. In this disclosure, the Al content is specified in terms of acid-soluble Al (also referred to as "Sol. Al" or the like).

### Ni: 0.40 % to 2.00 %

Ni is an element useful for improving the strength and toughness of the steel plate and is also useful for improving the CTOD property of the weld zone. In order to obtain these effects, the added content of Ni needs to be 0.40 % or more. Ni is an expensive element, however, and excessive addition thereof also increases the likelihood of damage to the surface of the slab at the time of casting. Therefore, the upper limit of the Ni content is set to 2.00 %.

### Mo: 0.05 % to 0.50 %

Mo is an element that fulfills an important function in this disclosure, and adding an appropriate amount thereof is useful for increasing the strength of the steel plate. This effect is obtained by improving the quench hardenability and the temper softening resistance at the time of tempering. Furthermore, Mo maintains the complex precipitate formed by Mo, Ti, and Nb in a fine state, thereby strengthening thick material and controlling a reduction in toughness. In order to obtain these effects, the Mo content needs to be at least 0.05 %. An excessive Mo content, however, adversely affects the toughness of the thick material. Hence, the upper limit on the Mo content is set to 0.50 %. The Mo content is more preferably in the range of 0.08 % to 0.40 %, and even more preferably in the range of 0.16 % to 0.30 %.

### Nb: 0.005 % to 0.040 %

Nb forms an unrecrystallized zone of austenite in the low temperature region. Therefore, by performing rolling in such a temperature region, the structure of the steel plate can be refined and the toughness of the steel plate can be increased. Furthermore, Nb has the effect of improving the quench hardenability, and by being added in combination with Mo and Ti, Nb has the effect of improving the softening resistance at the time of tempering. Nb is also a useful element for improving the strength of the steel plate. In order to obtain these effects, the Nb content needs to be at least 0.005 %. When the Nb content exceeds 0.040 %, however, the toughness deteriorates. Hence, the upper limit on the Nb content is set to 0.040 %, preferably 0.035 %.

### Ti: 0.005 % to 0.025 %

Ti is precipitated as TiN when molten steel solidifies, which suppresses coarsening of austenite in the weld zone, thus contributing to improvement in the toughness of the weld zone. Furthermore, by being added in combination with Mo and Nb, Ti has the effect of improving the softening resistance at the time of tempering. When the Ti content is less than 0.005 %, however, such an effect is small. On the other hand, when the Ti content exceeds 0.025 %, TiN coarsens, and it is not possible to obtain the effect of improving the toughness of the steel plate and the weld zone. Therefore, the Ti content is set in the range of 0.005 % to 0.025 %.

### N: 0.0020 % to 0.0050 %

N reacts with Ti and Al to form precipitates. Crystal grains are thereby refined, and the toughness of the steel plate is improved. Furthermore, N is a necessary element for forming TiN which suppresses coarsening of the structure of the weld zone. In order to obtain such effects, the N content needs to be set to 0.0020 % or more. On the other hand, when the N content exceeds 0.0050 %, solute N markedly degrades the toughness of the steel plate and the weld zone and leads to a deterioration in strength due to a reduction in solute Nb caused by generation of complex precipitates of Ti and Nb. Therefore, the upper limit on the N content is set to 0.0050 %.

### Ca: 0.0005 % to 0.0050 %

Ca is an element that improves toughness by fixing S. In order to obtain this effect, the Ca content needs to be at least 0.0005 %. On the other hand, Ca content exceeding 0.0050 % causes saturation of the effect. Therefore, Ca is added in the range of 0.0005 % to 0.0050 %.

### O: 0.0035 % or less

If the O content exceeds 0.0035 %, the toughness of the steel plate deteriorates. Hence, the O content is set to 0.0035 % or less, preferably 0.0028 % or less. The O content is preferably as small as possible, but considering factors such as refining cost, the lower limit may be approximately 0.0010 %.

### Ceq: 0.420 % to 0.520 %

When Ceq specified by the formula below is less than 0.420 %, a thick material strength of 460 MPa grade cannot be obtained. On the other hand, if Ceq exceeds 0.520 %, the weldability of the thick material and the toughness of the weld zone deteriorate. Hence, Ceq is set to 0.520 % or less. Ceq is preferably in the range of 0.440 % to 0.520 %. In the formula below, [M] represents the content (mass%) of element "M" in steel. Elements that are not included are calculated as zero. $Ceq = \left[C\right] + \left[Mn\right] / 6 + \left(\left[Cu\right]+\left[Ni\right]\right) / 15 + \left(\left[Cr\right]+\left[Mo\right]+\left[V\right]\right) / 5$

### [Ti]/[N]: 1.5 to 4.0

When the value of [Ti]/[N] is less than 1.5, the amount of TiN formed decreases, and solute N not forming TiN degrades the toughness of the weld zone. On the other hand, when the value of [Ti]/[N] exceeds 4.0, TiN is coarsened to degrade the toughness of the weld zone. Therefore, the value of [Ti]/[N] is set in the range of 1.5 to 4.0, and preferably 1.8 to 3.5.$0 < \left\{\left[Ca\right]-\left(0.18+130\times \left[Ca\right]\right)\times \left[O\right]\right\} / 1.25 / \left[S\right] < 1.5$ The expression {[Ca] - (0.18 + 130×[Ca])×[O]}/1.25/[S] is a value representing the Atomic Concentration Ratio (ACR) of Ca and S, which are effective for sulfide morphological control, and can be adjusted by controlling the amount of Ca added and the amount of dissolved oxygen in the molten steel at the time of addition to be within appropriate ranges. The sulfide morphology can be estimated by this ACR value, but in this disclosure, the ACR value is specified as an index in order to finely disperse CaS which does not dissolve even at high temperatures and which acts as nuclei for ferrite transformation.

When the ACR value is 0 or less, CaS is not crystallized. Consequently, S is precipitated in the form of MnS only, which easily dissolves in the heat-affected zone, making it impossible to obtain ferrite product nuclei. Furthermore, the MnS precipitated alone is elongated during rolling and causes degradation in the toughness of the steel plate. Therefore, in this disclosure, the ACR value needs to exceed zero.

On the other hand, when the ACR value is 1.5 or more, the proportion of oxides among Ca-based inclusions increases, and the proportion of sulfides that function as nucleation sites decreases, making it impossible to obtain the effect of improving toughness. Therefore, in this disclosure, the ACR value needs to be less than 1.5.

Accordingly, by controlling the ACR value to exceed 0 and be less than 1.5, complex sulfides mainly composed of CaS can be formed effectively and caused to function effectively as ferrite nucleation sites. The ACR value is preferably in the range of 0.15 to 1.30, and more preferably in the range of 0.20 to 1.00. $5.5 {\left[C\right]}^{\left(4/3\right)} + 15 \left[P\right] + 0.90 \left[Mn\right] + 0.12 \left[Ni\right] + 7.9 {\left[Nb\right]}^{\left(1/2\right)} + 0.53 \left[Mo\right] \leq 3.70$

The value of the left-hand side of the formula above (5.5[C]^{(4/3)} + 15[P] + 0.90[Mn] + 0.12[Ni] + 7.9[Nb]^{(1/2)} + 0.53[Mo]) is the hardness index of the central segregation area formed by components that are likely to be concentrated in the central segregation area and is referred to below as the Ceq* value.

Since the CTOD test is carried out over the entire thickness of a steel plate, test pieces include central segregation. In the case where the composition concentration in the central segregation is significant, a hardened region occurs in the heat-affected zone. Therefore, a good value cannot be obtained in the CTOD test.

Therefore, in this disclosure, by controlling the Ceq* value to be in an appropriate range, an excessive increase in hardness in the central segregation area can be suppressed, and an excellent CTOD property can be obtained even in the weld zone of a thick steel plate.

The appropriate range of the Ceq* value has been experimentally obtained. When the Ceq* value exceeds 3.70, the CTOD property is degraded. Therefore, the Ceq* value is set to be 3.70 or less, and preferably 3.50 or less. No lower limit is placed on the Ceq* value, but considering factors such as productivity, preferably the lower limit is approximately 2.2.

In this disclosure, in addition to the above-described essential elements, at least one selected from the group consisting of Cu: less than 0.7 %, Cr: 0.1 % to 1.0 %, and V: 0.005 % to 0.05 % may be added to increase quench hardenability.

### Cu: less than 0.7 %

Adding Cu improves the strength of the steel plate. If the content of Cu exceeds 0.7 %, however, the hot ductility deteriorates. Therefore, the Cu content is limited to 0.7 % or less. The Cu content is preferably 0.1 % to 0.6 %.

### Cr: 0.1 % to 1.0 %

Cr is an element effective in increasing the strength of the steel plate. In order to obtain this effect, the Cr content is set to 0.1 % or more. An excessively high Cr content, however, adversely affects toughness. Therefore, the Cr content is preferably 0.1 % to 1.0 %, and more preferably 0.2 % to 0.8 %, when included.

### V: 0.005 % to 0.05 %

V is an element that is effective in improving the strength and toughness of the steel plate at a content of 0.005 % or more. Setting the V content to exceed 0.05 %, however, leads to deterioration of toughness. Therefore, the V content is preferably 0.005 % to 0.05 % when included.

In this disclosure, in addition to the above-described essential elements, at least one selected from the group consisting of Mg: 0.0002 % to 0.0050 % and a REM: 0,0010 % to 0.0200 % may be added to increase the HAZ toughness.

Mg and REM are elements having the effect of improving the toughness of steel via the dispersion of oxides. In order to bring out such an effect, the Mg content is set to 0.0002 % or more, and the REM content to 0.0010 % or more. On the other hand, Mg content exceeding 0.0050 % and REM content exceeding 0.0200 % merely causes saturation of this effect. Accordingly, when adding these elements, the content is preferably set in the above-mentioned ranges. The Mg content is more preferably 0.0005 % to 0.0020 %, and the REM content is more preferably 0.0020 % to 0.0150 %.

Components other than the above-mentioned chemical composition are Fe and incidental impurities. In particular, when the steel plate is cooled from the austenite region, B exists in a segregated manner at austenite grain boundaries, suppresses ferrite transformation, and generates bainite structures that include a large amount of M-A. Hence, B has the disadvantage of making the structure brittle particularly in the heat-affected zone. Accordingly, in this disclosure, the content of B in the steel plate needs to be kept below 0.0003 %.

In the steel plate, the size of precipitates needs to change little before and after PWHT, and the strength and toughness of the steel plate need to be maintained. FIG. 1 illustrates the relationship between (i) the precipitate size and precipitate composition after PWHT and (ii) the change in strength and toughness before and after PWHT (ΔTS, ΔvTrs), and FIG. 2 illustrates TEM replica observation and EDX analysis results for precipitates in steel.

From the perspective of stability, the change in strength and in toughness before and after PWHT respectively need to satisfy the following ranges: ΔTS of 5 MPa to -15 MPA, and ΔvTrs of 10 °C to -5 °C. In order to satisfy these ranges, it is clear from FIG. 1 that the mean size of the precipitates needs to be kept to 20 nm or less, and that the Ti content (represented as [Ti]), the Nb content (represented as [Nb]), and the Mo content (represented as [Mo]) in the precipitates need to satisfy the relationship [Nb]/([Ti] + [Nb] + [Mo]) ≥ 0.3.

As is clear from Table I, which lists the EDX analysis results for precipitates in steel in FIG. 2, the above-mentioned precipitates are Ti, Nb, and Mo precipitates. Since it suffices for the relationship [Nb]/([Ti] + [Nb] + [Mo]) ≥ 0.3 to be satisfied, the precipitates need to be at least Nb precipitates, whereas Ti and Mo precipitates may be included in any range that satisfies this relationship. In this disclosure, having an excellent PWHT property refers to ΔTS being in the range of 5 MPa to -15 MPa, and ΔvTrs being in the range of 10 °C to -5 °C. The precipitates in this disclosure (complex precipitates) are Mo, Ti, and Nb precipitates. Specifically, these precipitates are carbides, nitrides, or carbonitrides of Mo, Ti, and Nb, or a mixture thereof.

### [Table 1]

**Table 1**

| Measuring Point No. | Ti (mass%) | Nb (mass%) | Mo (mass%) | [Nb]/([Ti]+[Nb]+[Mo]) |
|---|---|---|---|---|
| 5 | 15.51 | 82.1 | 2.39 | 0.821 |
| 6 | 27.63 | 72.37 | - | 0.724 |
| 7 | 20.52 | 79.48 | - | 0.795 |
| 8 | 20.92 | 65.6 | 13.48 | 0.656 |

### [Method of Determining Precipitate Particle Size]

The method of determining the precipitate particle size in this disclosure is in accordance with the TEM replica method. Specifically, after appropriately collecting the precipitate zone of Ti, Nb, and Mo carbides from the steel, the average equivalent circular diameter was determined using image processing on an observation made at 100,000X over four fields of view and taken as the particle size of the precipitates. In this disclosure, the lower limit on the measurement target for precipitate size was set to 2 nm. The reason is that precipitates with a precipitate size smaller than 2 nm are hard to measure.

Next, our method for manufacturing steel will be described. Our steel is preferably manufactured with the method of manufacturing described below.

Molten steel adjusted to have a chemical composition within the above-described ranges is prepared by steelmaking with an ordinary method using a converter, an electric heating furnace, a vacuum melting furnace, or the like. Next, after forming the molten steel into a slab by continuous casting, the slab is hot rolled to a desired plate thickness. The result is then cooled, and as necessary, tempered. During the hot rolling of this disclosure, the slab heating temperature and rolling reduction are prescribed.

In this disclosure, unless otherwise noted, the temperature conditions on the steel plate are prescribed by the temperature at the central portion in the plate thickness direction of the steel plate. The temperature at the central portion in the plate thickness direction is determined from the plate thickness, the surface temperature, the cooling conditions, and the like by simulation calculation or the like. For example, the temperature at the central portion in the plate thickness direction may be determined by calculating the temperature distribution in the plate thickness direction using the finite difference method.

### Slab reheating temperature: 950 ° C to 1150 ° C

The slab reheating temperature is set to 950 °C or higher in order to remove casting defects in the slab reliably with hot rolling. If the slab is reheated to a temperature exceeding 1150 °C, however, the austenite crystallized grains coarsen, causing the toughness of the steel plate to degrade. Hence, the upper limit on the slab reheating temperature is set to 1150 °C.

### Cumulative rolling reduction of hot rolling in a temperature range of 900 °C or higher: 30 % or higher

In order to render casting defects harmless by pressure bonding and to provide austenite grains with a fine microstructure by recrystallization, the cumulative rolling reduction of hot rolling in a temperature range of 900 °C or higher is set to 30 % or higher. The reason is that if the cumulative rolling reduction is less than 30 %, coarse grains formed during reheating remain and adversely affect the toughness of the steel plate. No upper limit is placed on the cumulative rolling reduction of hot rolling in a temperature range of 900 °C or higher, but in industrial terms, the upper limit is approximately 95 %.

### Cumulative rolling reduction of hot rolling in a temperature range of less than 900 °C: 30 % to 70 %

In this temperature range, the rolled austenite grains do not sufficiently recrystallize. Therefore, austenite grains that remain flattened after rolling constitute a state of high internal distortion that includes numerous defects, such as an internal distortion zone. These austenite grains act as the driving force for ferrite transformation and encourage phase transformation.

If the cumulative rolling reduction is less than 30 %, however, accumulation of internal energy in the distortion zone is insufficient, making it difficult for ferrite transformation to occur and reducing the toughness of the steel plate. Conversely, if the cumulative rolling reduction exceeds 70 %, generation of polygonal ferrite is encouraged, making high strength and high toughness incompatible. Accordingly, in this disclosure, the cumulative rolling reduction of hot rolling in a temperature range of less than 900 °C is set in the range of 30 % to 70 %.

### Cooling rate at least to 500 °C: 1.0 °C/s or higher

After hot rolling, accelerated cooling is performed at least to 500 °C at a cooling rate of 1.0 °C/s or higher. The reason is that if the cooling rate is less than 1.0 °C/s, sufficient strength of the steel plate is not obtained. Furthermore, if cooling is stopped at a higher temperature than 500°C, the proportion of ferrite and pearlite structure increases, making high strength and high toughness of thick material incompatible. While no lower limit is placed on the stop temperature of accelerated cooling, the steel is preferably cooled to room temperature.

### Tempering temperature: 450 °C to 650 °C

In this disclosure, when tempering the steel, a sufficient tempering effect is not obtained if the tempering temperature is less than 450 °C. On the other hand, when tempering at a temperature exceeding 650 °C, the precipitates may coarsen, lowering the toughness and the strength of the steel. Hence, a temperature exceeding 650 °C is not preferable.

The tempering in this disclosure more preferably uses induction heating, which suppresses coarsening of carbides during tempering. In this case, the tempering is preferably performed so that the temperature at the center of the steel plate calculated by a simulation using the finite difference method or the like is from 450 °C to 650 °C.

In this disclosure, when desired properties of the steel plate have been obtained, as for a TMCP steel plate or the like, the above-described tempering need not be performed.

Thick material in this disclosure has a thickness of 15 mm or greater. Accordingly, the thickness in this disclosure refers to a steel thickness of 15 mm or greater, but the effects of this disclosure are best obtained when the steel thickness is in a range of 40 mm to 100 mm. Manufacturing conditions other than the above-described manufacturing conditions on thick, high tensile strength steel may be in accordance with conventional methods.

In the thick, high tensile strength steel of this disclosure, coarsening of austenite grains in the heat-affected zone is suppressed while finely dispersing nuclei for ferrite transformation that do not dissolve even at high temperatures, thereby refining the structure of the heat-affected zone. High toughness is thus obtained. Also in an area reheated to a dual phase by the thermal cycle at the time of multilayer welding, the structure of the heat-affected zone due to initial welding is refined. Therefore, in the dual phase reheating area, the toughness of the non-transformed area can be improved, the austenite grains that undergo retransformation can be refined, and the extent of reduction in toughness can be reduced. Additionally, by generating fine complex precipitates of Ti, Nb, and Mo, a thick, high tensile strength steel plate is provided with an excellent CTOD property and PWHT property.

### EXAMPLES

Examples according to this disclosure are now described.

Using continuously-cast slabs with steel codes A to Z having the chemical composition listed in Table 2 as raw material, the hot rolling and heating listed in Table 3 were performed to produce thick steel plates with a thickness of 50 mm to 150 mm. The steel plates were evaluated by a tensile test in which JIS No. 4 test pieces were collected from the 1/2 position along the thickness of the steel plates, so that the longitudinal direction of each test piece was perpendicular to the rolling direction of the steel plate. The yield stress (YS) and tensile strength (TS) were then measured.

A Charpy impact test was also performed by collecting JIS No. 4 V-notch test pieces measuring 2 mm from the 1/2 position along the thickness of the steel plates, so that the longitudinal direction of each test piece was perpendicular to the rolling direction of the steel plate. The absorbed energy vE₋₄₀ °C at -40 °C was then measured. In these Examples, the base metal properties were evaluated as being good when all of the following relationships were satisfied: YS ≥ 460 MPa, TS ≥ 570 MPa, and vE₋₄₀ °C ≥ 200 J.

The toughness of the weld zone was evaluated by producing a multilayer fill weld joint, using a single bevel groove, by submerged arc welding having a welding heat input of 35 kJ/cm and measuring the absorbed energy vE₋₄₀ °C at -40 °C with a Charpy impact test, using the weld bond on the straight side at the 1/2 position along the thickness of the steel plates as the notch position for the test. The toughness of the weld zone was determined to be good when the mean for three tests satisfied the relationship vE₋₄₀ °C ≥ 150 J.

Using the weld bond at the straight side as the notch position for the CTOD test pieces, the CTOD value at -10 °C, i.e. δ-10 °C, was measured. The CTOD property of the weld joint was determined to be good when the minimum of the CTOD value (δ-10 °C) over three tests was 0.5 mm or greater.

Furthermore, the precipitate zone in the steel was collected by the TEM replica method, and the average equivalent circular diameter was determined using image processing on an observation made at 100,000X over four fields of view. Precipitates with a particle size near the mean were selected by EDX, the precipitate composition thereof was determined, and [Nb]/([Ti]+[Nb]+[Mo]) was determined as the mean of three precipitates.

Regarding the change in base metal properties after PWHT, ΔTS (TS(after PWHT) - TS(before PWHT)) and ΔvTrs (vTrs(after PWHT) - vTrs(before PWHT)) were determined. PWHT was performed by maintaining the steel at 580 °C for four hours, with temperature raising and lowering rates of 70 °C/h.

Table 3 illustrates the hot rolling conditions, heat treatment conditions, base metal properties, the results of the above-described Charpy impact test and CTOD test on the weld zone, the precipitate size/composition, and the change in base metal properties after PWHT.

As listed in Table 2, steel codes A to E represent steel conforming to this disclosure, whereas steel codes F to Z represent comparative steel in which one of the steel components is outside of the range of this disclosure. Sample Numbers 1, 2, 5, 6, 8, and 11 in Table 3 are all Examples for which the results of the Charpy impact test on the weld bond, the results of the three-point bending CTOD test on the weld bond, the precipitate size/composition in the steel plate, and the PWHT property all satisfy the targets.

Conversely, in Sample Numbers 3, 4, 7, 9, 10, and 12 to 31, at least one of the steel plate components, the manufacturing conditions, and the precipitate size/composition fall outside of the ranges of this disclosure, and one of the base metal properties, the results of the Charpy impact test on the weld bond, the results of the three-point bending CTOD test on the weld bond, and the PWHT property does not satisfy the target. In Table 3, entries marked with a horizontal line are entries for which measurement was not possible.

The steel of the Examples according to this disclosure has both excellent strength and toughness of the steel plate, as the yield stress (YS) of the steel plate is 460 MPa or higher, and the Charpy absorbed energy (vE₋₄₀ °C) is 200 J or higher. Furthermore, in the weld joint bond, vE₋₄₀ °C is 150 J or higher, and the CTOD value is 0.5 mm or higher, thus also providing excellent toughness in the heat-affected zone. When the mean particle size of the precipitates is 20 µm or less and [Nb]/([Ti]+[Nb]+[Mo]) ≥ 0.3, then the base metal property after PWHT is also excellent. By contrast, in the Comparative Examples outside of the ranges of this disclosure, only steel plates for which one of the above-described properties was inferior could be achieved.

## Claims

1. A steel plate, comprising:
a chemical composition consisting of, by mass%,
C: 0.020 % to 0.090 %,
Si: 0.01 % to 0.35 %,
Mn: 1.40 % to 2.00 %,
P: 0.008 % or less,
S: 0.0035 % or less,
Al: 0.010 % to 0.060 %,
Ni: 0.40 % to 2.00 %,
Mo: 0.05 % to 0.50 %,
Nb: 0.005 % to 0.040 %,
Ti: 0.005 % to 0.025 %,
N: 0.0020 % to 0.0050 %,
Ca: 0.0005 % to 0.0050 %, and
O: 0.0035 % or less,
Ceq specified by formula (1) below being in a range of 0.420 % to 0.520 %, formulas (2), (3), and (4) below being satisfied, optionally at least one selected from the group consisting of, by mass%,
Cu: less than 0.7 %,
Cr: 0.1 % to 1.0 %,
V: 0.005 % to 0.05 %
Mg: 0.0002 % to 0.0050 % and
a REM: 0.0010 % to 0.0200 %, and the balance being Fe and incidental impurities including B of less than 0.0003 %; and
precipitates including Ti, Nb, and Mo and having a mean particle size of 2 nm or more and 20 nm or less, wherein [Nb]/([Ti] + [Nb] + [Mo]) ≥ 0.3, where [Ti] is the Ti content in the precipitates, [Nb] is the Nb content in the precipitates, and [Mo] is the Mo content in the precipitates: $Ceq = \left[C\right] + \left[Mn\right] / 6 + \left(\left[Cu\right]+\left[Ni\right]\right) / 15 + \left(\left[Cr\right]+\left[Mo\right]+\left[V\right]\right) / 5$ $1.5 \leq \left[Ti\right] / \left[N\right] \leq 4.0$ $0 < \left\{\left[Ca\right]-\left(0.18+130\times \left[Ca\right]\right)\times \left[O\right]\right\} / 1.25 / \left[S\right] < 1.5$ $5.5 {\left[C\right]}^{\left(4/3\right)} + 15 \left[P\right] + 0.90 \left[Mn\right] + 0.12 \left[Ni\right] + 7.9 {\left[Nb\right]}^{\left(1/2\right)} + 0.53 \left[Mo\right] \leq 3.70$ where [M] is the content of element M by mass%, and
a thickness of the steel plate is 15 mm or more, and wherein the steel plate has
a YS of 460 MPa or more,
a TS of 570 MPa or more,
a Charpy absorbed energy vE₋₄₀ °C of 200 J or more,
a ΔTS of 5 MPa to -15 MPa, and
a ΔvTrs of 10 °C to -5 °C,
where ΔTS is the change in tensile strength in the base metal before and after post weld heat treatment, and ΔvTrs is the change in toughness in the base metal before and after post weld heat treatment.

2. A method for manufacturing a steel plate according to claim 1, the method comprising:
heating steel having the chemical composition according to claim 1 to 950 °C to 1150 °C;
subsequently subjecting the steel to hot rolling at a cumulative rolling reduction of 30 % or higher in a temperature range of 900 °C or higher and a cumulative rolling reduction of 30 % to 70 % in a temperature range of less than 900 °C;
subsequently cooling the steel at least to 500 °C at the central portion in the plate thickness direction of the steel plate with a cooling rate of 1.0 °C/s or higher,
and further optionally comprising tempering at 450 °C to 650 °C after the cooling.

## Patentansprüche

1. Stahlblech, das umfasst:
eine chemische Zusammensetzung, die in Masse-% aus
0,020 % bis 0,090 % C,
0,01 % bis 0,35 % Si,
1,40 % bis 2,00 % Mn,
0,008 % oder weniger P,
0,0035 % oder weniger S,
0,010 % bis 0,060 % Al,
0,40 % bis 2,00 % Ni,
0,05 % bis 0,50 % Mo,
0,005 % bis 0,040 % Nb,
0,005 % bis 0,025 % Ti,
0,0020 % bis 0,0050 % N,
0,0005 % bis 0,0050 % Ca sowie
0,0035 % oder weniger O,
Ceq, vorgegeben durch Formel (1), das in einem Bereich von 0,420 % bis 0,520 % liegt, wobei die Formeln (2), (3) und (4) erfüllt sind, optional wenigstens einem Element, das aus der Gruppe ausgewählt wird, die in Masse-% aus
weniger als 0,7 % Cu,
0,1 % bis 1,0 % Cr,
0,005 % bis 0,05 % V,
0,0002 % bis 0,0050 % Mg sowie
0,0010 % bis 0,0200 % eines REM besteht, wobei der Rest Fe und zufällige Verunreinigungen einschließlich B von weniger als 0,0003 % sind; sowie
Ausfällungen besteht, die Ti, Nb und Mo enthalten und eine mittlere Teilchengröße von 2 nm oder mehr und 20 nm oder weniger haben, wobei [Nb]/([Ti] + [Nb] + [Mo]) ≥ 0,3, dabei [Ti] der Ti-Gehalt in den Ausfällungen ist, [Nb] der Nb-Gehalt in den Ausfällungen ist und [Mo] der Mo-Gehalt in den Ausfällungen ist: $Ceq = \left[C\right] + \left[Mn\right] / 6 + \left(\left[Cu\right]+\left[Ni\right]\right) / 15 + \left(\left[Cr\right]+\left[Mo\right]+\left[V\right]\right) / 5$ $1,5 \leq \left[Ti\right] / \left[N\right] \leq 4,0$ $0 < \left\{\left[Ca\right]-\left(0,18+130\times \left[Ca\right]\right)\times \left[O\right]\right\} / 1,25 / \left[S\right] < 1,5$ $5,5 {\left[C\right]}^{\left(4/3\right)} + 15 \left[P\right] + 0,90 \left[Mn\right] + 0,12 \left[Ni\right] + 7,9 {\left[Nb\right]}^{\left(1/2\right)} + 0,53 \left[Mo\right] + 0,53 \left[Mo\right] \leq 3,70$ wobei [M] der Gehalt an Element M in Masse-% ist, und
eine Dicke des Stahlblechs 15 mm oder mehr beträgt, und wobei das Stahlblech
eine Streckfestigkeit von 460 MPa oder mehr;
eine Zugfestigkeit von 570 MPa oder mehr;
eine im Kerbschlagbiegeversuch nach Charpy absorbierte Energie vE₋₄₀ °C von 200 J oder mehr,
eine ΔTS von 5 MPa bis -15 MPa, sowie
eine ΔvTrs von 10 °C bis -5 °C hat,
wobei ΔTS die Änderung der Zugfestigkeit in dem Grundmetall vor und nach Wärmebehandlung nach dem Schweißen ist und ΔvTrs die Änderung der Zähigkeit in dem Grundmetall vor und nach der Wärmebehandlung nach dem Schweißen ist.

2. Verfahren zum Herstellen eines Stahlblechs nach Anspruch 1, wobei das Verfahren umfasst:
Erhitzen von Stahl, der die chemische Zusammensetzung nach Anspruch 1 hat, auf 950 °C bis 1150 °C;
anschließendes Warmwalzen des Stahls bei einer kumulativen Walzreduktion von 30 % oder mehr in einem Temperaturbereich von 900 °C oder darüber und einer kumulativen Walzreduktion von 30 % bis 70 % in einem Temperaturbereich unter 900 °C;
anschließendes Abkühlen des Stahls auf wenigstens 500 °C im mittleren Abschnitt der Richtung der Blechdicke des Stahlblechs mit einer Abkühlgeschwindigkeit von 1,0 °C/s oder darüber,
und wobei es des Weiteren optional Anlassen bei 450 °C bis 650 °C nach dem Abkühlen umfasst.

## Revendications

1. Plaque d'acier, comprenant :
une composition chimique constituée de, en % en masse,
C : 0,020 % à 0,090 %,
Si : 0,01 % à 0,35 %,
Mn : 1,40 % à 2,00 %,
P : 0,008 % ou moins,
S : 0,0035 % ou moins,
Al : 0,010 % à 0,060 %,
Ni : 0,40 % à 2,00 %,
Mo : 0,05 % à 0,50 %,
Nb : 0,005 % à 0,040 %,
Ti : 0,005 à 0,025 %,
N : 0,0020 % à 0,0050 %,
Ca : 0,0005 % à 0,0050 %, et
O : 0,0035 % ou moins,
Ceq spécifié par la formule (1) ci-dessous se situant dans une plage de 0,420 % à 0,520 %, les formules (2), (3) et (4) ci-dessous étant satisfaites, facultativement au moins l'un choisi parmi le groupe constitué de, en % en masse,
Cu : moins de 0,7 %,
Cr : 0,1 % à 1,0 %,
V : 0,005 % à 0,05 %
Mg : 0,0002 % à 0,0050 % et
REM: 0,0010 % à 0,0200 %, le reste étant Fe et des impuretés accidentelles incluant B à moins de 0,0003 % ; et
de précipités comprenant Ti, Nb, et Mo et ayant une taille moyenne de particules de 2 nm ou plus et de 20 nm ou moins, dans laquelle [Nb]/([Ti] + [Nb] + [Mo]) ≥ 0,3,
où [Ti] est la teneur en Ti dans les précipités, [Nb] est la teneur en Nb dans les précipités, et [Mo] est la teneur en Mo dans les précipités : $Ceq = \left[C\right] + \left[Mn\right] / 6 + \left(\left[Cu\right]+\left[Ni\right]\right) / 15 + \left(\left[Cr\right]+\left[Mo\right]+\left[V\right]\right) / 5$ $1,5 \leq \left[Ti\right] / \left[N\right] \leq 4,0$ $0 < \left\{\left[Ca\right]-\left(0,18+130\times \left[Ca\right]\right)\times \left[O\right]\right\} / 1,25 / \left[S\right] < 1,5$ $5,5 {\left[C\right]}^{\left(4/3\right)} + 15 \left[P\right] + 0,90 \left[Mn\right] + 0,12 \left[Ni\right] + 7,9 {\left[Nb\right]}^{\left(1/2\right)} + 0,53 \left[Mo\right] \leq 3,70$ où [M] est la teneur en l'élément M en % en masse, et
une épaisseur de la plaque d'acier est de 15 mm ou plus, et dans laquelle la plaque d"acier présente
une YS de 460 MPa ou plus,
une TS de 570 MPa ou plus,
une énergie absorbée par Test Charpy vE₋₄₀ °C de 200 J ou plus,
un ΔTS de 5 MPa à -15 MPa, et
un ΔvTrs de 10 °C à -5 °C,
où ΔTS est le changement de résistance à la traction dans le métal de base avant et après traitement thermique post-soudure, et ΔvTrs est le changement de robustesse dans le métal de base avant et après traitement thermique post-soudure.

2. Procédé de fabrication d'une plaque d'acier selon la revendication 1, le procédé comprenant les étapes consistant à :
chauffer un acier ayant la composition chimique selon la revendication 1 entre 950 °C et 1150 °C ;
soumettre ensuite l'acier à un laminage à chaud à une réduction de laminage cumulative de 30 % ou plus dans une plage de température de 900 °C ou plus et une réduction de laminage cumulative de 30 % à 70 % dans une plage de température inférieure à 900 °C ;
refroidir ensuite l'acier à au moins 500 °C au niveau de la partie centrale dans la direction d'épaisseur de plaque de la plaque d'acier à une vitesse de refroidissement de 1,0 °C/s ou plus,
et comprenant facultativement en outre une trempe entre 450 °C et 650 °C après le refroidissement.
